

July 28, 1959

M. VAN DAM

2,897,090

HEAT-SENSITIVE COPYING PAPER

Filed April 11, 1957

FIG. 1.



FIG. 2.



INVENTOR

MAX VAN DAM

BY *Samuel J. Stoeck*

ATTORNEY

1

2,897,090

**HEAT-SENSITIVE COPYING PAPER**

Max Van Dam, Newton, N.J., assignor to Anken Chemical & Film Corporation, Newton, N.J.

Application April 11, 1957, Serial No. 652,103

12 Claims. (Cl. 117—36)

This invention relates to an improved heat-sensitive duplicating paper useful in preparing copies of printed matter or the like.

More specifically, this invention is concerned with heat-sensitive coating and coated sheet materials designed for preparing copies of printed matter or other graphic subject matter by exposure to high intensity irradiation and without subsequent developing or fixing operations.

Heat-sensitive coatings of this type, for preparing copies by direct exposure to high intensity irradiation without further treatment, are known, and several have been described, as in Miller and Clark, U.S. Patents 2,663,654, issued December 22, 1953, and 2,710,263, issued June 7, 1955; also Miller, U.S. Patent 2,740,896, issued April 3, 1956.

Significant limitations or disadvantages exist in the coatings for this purpose heretofore described however. Perhaps the most important of these is the lack of black and white contrast in copies made with these coatings. In most instances, the white is not white and the black not black. Frequently, the copying paper shows a buff background rather than white; and by virtue of the components used, a violet or blue image results instead of a neutral black. While heat-sensitive coatings with a white background are known, these produce an image which is most often dark brownish rather than black. True black and white copies have not been achieved.

Lack of sharp outline in black and white copies is also encountered in these previously described coatings. The boundary between the light background and the image is insufficiently distinct in the copies resulting from them; a spreading or bleeding effect occurs; the copied image thus is unsharp or blurred.

Another major limitation of prior coatings is the narrow range of exposure conditions which will produce a satisfactory readable copy. Exposure to the optimum quantity of radiant energy may give reasonably acceptable results; but minor variations in the amount of irradiation give poor or unreadable copies. Underexposure to a relatively small degree produces too light a copy with insufficient contrast; overexposure to the same extent produces a copy with too dark a background.

A still further drawback to previously proposed coatings is that their components are so reactive and unstable toward each other that they must be ground or mixed separately, and in many instances, even applied to the sheet material as separate multiple coatings.

Still another drawback is the sensitivity of prior coatings to impurities such as small particles of chemical materials and coarse dust. Such impurities show up as dark spots on the copy.

It is, therefore, an object of my invention to provide novel and useful compositions as coatings for copying paper which can produce neutral black and white copies.

Another object of my invention is to provide compositions of a heat-sensitive material which will produce

2

satisfactory copies when subjected to relatively widely varied quantities of radiant energy.

Another object of my invention is to provide compositions of a heat-sensitive coating which will afford copies sharp and clear, with distinct boundaries between the image and the background.

Still another object of my invention is to provide compositions which can be ground and mixed in one operation, and applied to the sheet material as a single coating.

A further object is the provision of heat-sensitive copying paper which is not oversensitive to impurities.

In conventional photography, the black image and the gray tones consist of metallic silver, reduced to the metal state from silver salts by the action of light and, of course, a suitable developer. The present invention is based on the discovery that under certain conditions black and neutral gray tones can be formed of metallic bismuth, suitably reduced to the metal state from bismuth salts. The requisite conditions are similar to those for the well-known reaction in aqueous alkaline solution whereby a bismuth salt can be reduced by sodium stannite to metallic bismuth.

In place of sodium stannite or other tin salt and an alkali hydroxide, which are unstable and impractical (sodium stannite forms stannate in air, and the hydroxide changes into carbonate), this invention makes primary use of derivatives of tin and organic alkaline compounds.

Bismuth is the key ingredient in this process, as silver is the key ingredient in photographic processes. The starting point is a bismuth salt and the process reduces it to metallic bismuth. Reduction takes place only in the presence of heat.

The required ingredients for a coating composition made in accordance with this invention are the following:

- (1) A bismuth salt.
- (2) A reducing agent.
- (3) A suitable medium.
- (4) A reaction regulator.
- (5) A binder (optional).

(1) Bismuth salt: The bismuth compound may be the salt of an inorganic or organic acid. For example, suitable inorganic salts would be bismuth borate, and bismuth oxychloride. Suitable organic salts would be bismuth subsalicylate and bismuth benzoate.

(2) A reducing agent: A suitable reducing agent would be a tin derivative, either inorganic or organic. Illustrative inorganic reducing agents are stannous sulfate, tin hydroxide and other tin derivatives but other inorganic reducing agents may also be used, such as sodium hydrosulfite. Suitable organic tin derivatives are piperidine-tin chloride, semicarbazide-tin sulfate, di-phenylamine-tin chloride, methylamine-tin sulfate, aniline-tin sulfate, tin oxalate, tin tartrate, tin citrate, tin glycolate, and tin formate. These organic tin derivatives are illustrative of the various derivatives of this nature which have been made from semicarbazide, hydrazine, pyridine, aniline, methylamine, triethylamine, triethanolamine, triisopropanolamine, piperidine, di-phenylamine.

(3) A suitable medium: An alkaline medium, preferably organic, is preferred and suitable compounds are: semicarbazide, heterocyclic base and their derivatives such as amino-pyridine amines and amino derivatives, e.g. ethanolamines. Liquid alkaline substances can be used, preferably by converting them into new solid compounds through addition or condensation with weakly acid-reacting compounds. As liquid compounds may be used: Methylamine, dimethylamine, aniline, pyridine,

quinoline, hydrazine, triethylamine, triethanolamine, piperidine. They may be combined with: Oxalic acid, tartaric acid, salicylic acid, benzoic acid.

(4) Reaction regulator: Regulators may be used to control the spread of the reaction and hence the sensitivity or range of the coating to different amounts of radiant energy. As regulators, low-melting materials are used, preferably but not necessarily organic alkaline compounds. Suitable compounds for this purpose have been found to be benzylthiocyanate, chlorophenol, cinnamyl alcohol, o-cresol, diphenylamine, hexadecanol, hexadecylamine, p-toluidine, triphenyl phosphate, o-vanillin, amino diphenylamine, p-hydroxy diphenylamine and phenyl diethanolamine. The dry ingredients of the mixture do not react quickly and these last listed materials are used to lower the melting point.

(5) Binder: A suitable binder in solution, and coating modifiers such as plasticizers, softeners, etc., may be used. Typical binders suitable for the purposes of this invention are the following: cellulose acetate, cellulose acetobutyrate, cellulose nitrate, ethyl cellulose, rubber and chlorinated rubber and ethyl hydroxyethyl cellulose.

As has above been indicated, the key element in the entire process is bismuth but since we start with a bismuth compound, it is necessary to utilize a reducing agent. Since the reaction will take place best in a suitable medium, the medium is also provided. Nonetheless, since the reaction may also take place without such medium, the latter is employed solely to expedite and facilitate the reaction. By the same token, a regulator is also used to control the reaction in order to provide sharply defined results but in the absence of such regulator, the reaction would still take place and with good results, falling short, however, of the excellent results attained with the use of a regulator. The use of a binder is not essential and when used a small amount suffices. The binder helps to prevent setting of the materials during the coating process and keeps them in suspension. It also provides better adhesion to the paper.

It will be apparent from the foregoing, that the two key ingredients of the present invention are a bismuth compound and a reducing agent. But the other three ingredients are used to improve the process and for improved results. Aside from the fact that these three ingredients are not absolutely essential in the reaction, there may also be overlapping which would reduce their number without loss of their respective functions. For example, the alkaline medium and the regulator may overlap in that the regulator is preferably an organic alkaline compound. Consequently, it would not only perform the function of controlling the reaction but it would also supply the alkaline medium in which the reaction would take place.

Compositions prepared in accordance with this invention may be applied as a coating to paper, film and other light-transmitting material, either transparent or translucent, and other sheet materials may be used providing that they are transparent to heat. The result is a heat-sensitive copy-medium. The invention is illustrated in the accompanying drawing, in which:

Fig. 1 shows the manner of use of a heat-sensitive copy-medium made in accordance with this invention, said copy-medium and the original to be copied being shown in section and the radiations from the heat source being represented by means of interrupted lines.

Fig. 2 is a plan view of said heat-sensitive copy-medium superimposed upon the original to be copied, said view following the exposure of said copy-medium and said original to radiant energy, one corner of said copy-medium being folded over to show the result of such exposure.

Referring now to Fig. 1 of the drawing, it will be observed that in the use of a heat-sensitive copy-medium in accordance with this invention, said copy-medium is superimposed upon and in contact with the original

which is to be copied. In the drawing, the heat-sensitive copy-medium is shown to consist of a light-transmitting base, such as a sheet of light-transmitting paper, covered with a heat-sensitive coating prepared in accordance with this invention.

The heat-sensitive copy-medium is superimposed upon and in contact with the original to be copied, said original being shown in the drawing as a sheet of paper or the like having printed, typewritten or written material applied thereto and indicated by the interrupted lines thereon.

Radiant energy is then applied through said heat-sensitive copy-medium to the original to be copied. This is done by the use of any suitable source of radiant energy, as for example an infra-red lamp as shown in Fig. 1 of the drawing. The interrupted lines between said infra-red lamp and said heat-sensitive copy-medium are intended to represent the radiations which emanate from said infra-red lamp.

More heat is generated by said radiant energy in the printed or other written matter on the original to be copied than in the blank spaces surrounding said printed or written matter, such heat being sufficient to cause the chemical reaction in the heat-sensitive coating herein described. The bismuth compound is reduced to metallic bismuth in the precise areas on the heat-sensitive copy-medium which correspond to the graphic material on the original to be copied, and the result is that an identical copy of said graphic material is formed on the heat-sensitive copy-medium and indicated in the drawing by the interrupted lines on the heat-sensitive copy-medium shown in Fig. 2.

The following coating compositions are given as specific examples illustrative of the invention and they are not to be considered restrictive or limitative of its scope:

## I

In a ball-mill was mixed the following mixture:

|                            | Grams |
|----------------------------|-------|
| Bismuth borate             | 2690  |
| Semicarbazide              | 2500  |
| Stannous sulfate anhydrous | 2150  |
| Diethanolamine             | 1200  |
| Cellulose acetate          | 200   |
| Methanol                   | 300   |
| Acetone                    | 1200  |
| Dichlorethane              | 500   |

After mixing, the mixture was uniformly spread by means of a doctor-blade onto a thin transparent paper and dried at room temperature.

The resulting sheet is suitable for use as a heat-sensitive copying paper.

## II

The following mixture was ball-milled and coated on light transmitting paper:

|                      | Grams |
|----------------------|-------|
| Bismuth oxychloride  | 2610  |
| Tin tartrate         | 2670  |
| Semicarbazide        | 2000  |
| Diphenylamine        | 2000  |
| Di iso propanolamine | 1000  |
| Ethyl cellulose      | 10    |
| Toluene              | 2250  |

## III

The following mixture was ball-milled and coated on light transmitting paper:

|                       | Grams |
|-----------------------|-------|
| Bismuth subsalicylate | 36    |
| Tin hydroxide         | 20    |
| Tri-isopropanolamine  | 19    |
| Polyvinylbutyral      | 25    |
| Semicarbazide         | 25    |
| Toluene               | 30    |

The following mixture was ball-milled and coated on translucent paper:

|                              |    |     |    |
|------------------------------|----|-----|----|
| Bismuth lactate              | g  | 36  | 5  |
| Semicarbazide-tin chloride   | g  | 34  |    |
| Semicarbazide                | g  | 15  |    |
| Hydrazine salicylate         | g  | 20  |    |
| Ethyl hydroxyethyl cellulose | g  | 1   |    |
| Toluene                      | ml | 50  | 10 |
| Ligroine                     | ml | 400 |    |

The following mixture was ball-milled and coated on transparent paper:

|                             | Grams |
|-----------------------------|-------|
| Bismuth subnitrate          | 2930  |
| Triethylamine-tin chloride  | 2910  |
| Semicarbazide               | 2500  |
| Ethyl paratoluene sulfonate | 1000  |
| Cellulose nitrate           | 200   |
| Acetone                     | 2300  |

It will be noted that organic tin derivatives are used in the foregoing examples. The following procedures may be used in producing these derivatives:

#### A. Preparation of piperidine-tin chloride

To a solution of 190 g. of anhydrous tin chloride in 500 ml. of water was added 85 g. of piperidine.

The white precipitate which formed was immediately filtered off, washed with water, methanol and dried.

Yield: 81 g. of piperidine-tin chloride.

#### B. Preparation of semicarbazide-tin sulfate

150 g. of semicarbazide dissolved in 230 ml. of water was added to a solution of 215 g. of anhydrous tin sulfate in 230 ml. of water.

The mixture warmed spontaneously and precipitate was formed. After standing for 2 hours the precipitate was filtered off, washed with water, then with methanol and dried.

Yield: 35 g. of semicarbazide-tin sulfate in the form of a white powder.

#### C. Preparation of diphenylamine-tin chloride

A solution of 338 g. of diphenylamine in 50 ml. of methanol was added to a solution of 190 g. of anhydrous tin chloride in 500 ml. of water; immediately a precipitate was formed. One liter of methanol was added to the slurry. The precipitate was filtered, washed with water and methanol.

Yield: 500 g. of diphenylamine-tin chloride in the form of a white powder.

#### D. Preparation of methylamine-tin sulfate

To a solution of 215 g. of anhydrous tin sulfate in 500 ml. of water was added 120 g. of a 25% solution of methylamine in water. The white precipitation which formed was immediately filtered off, washed with water, then with methanol and dried.

Yield: 60 g. of methylamine-tin sulfate in the form of a white powder.

#### E. Preparation of aniline-tin sulfate

To a solution of 107 g. of anhydrous tin sulfate in 250 ml. of water was added 93 g. of aniline. The precipitate which formed was filtered, washed with water, methanol and dried.

Yield: 130 g. of aniline-tin sulfate.

It will be noted that salts of weak acids and strong alkalines are used in a foregoing example.

The following procedures may be used in producing these components:

#### F. Preparation of hydrazine tartrate

To a solution of 150 g. of tartaric acid in 500 ml. of 75

methanol was added 50 g. of hydrazine monohydrate. The white precipitate which was formed immediately, was filtered, washed with methanol and dried.

Yield: 135 g. of hydrazine tartrate.

#### G. Preparation of hydrazine-salicylate

To a slurry of 151 g. of salicylic acid in 200 ml. of methanol was added: 67 g. of hydrazine monohydrate. The mixture warmed spontaneously and the salicylic acid went into solution. The methanol was evaporated on a steam bath. After cooling the residue solidified:

Yield: 190 g. of hydrazine salicylate.

The foregoing is illustrative of the basic principles of this invention and it will be understood that all of the examples above set forth are merely illustrative of the invention and not limitative thereof and that modifications and variations of these examples, as well as other examples involving other procedures and formulae producing the same or similar results may also be employed within the broad spirit of the invention and the broad scope of the claims.

I claim:

1. A heat-sensitive copying sheet for producing copies of printed or graphic subject matter by exposure of said sheet, in contact with said subject matter, to radiant energy, said copying sheet having applied thereto the combination of a bismuth compound and a tin derivative reducing agent capable of reacting with said bismuth compound in the presence of heat to produce metallic bismuth.

2. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound being a bismuth salt which is combined with a tin derivative reducing agent in an organic alkaline medium.

3. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound being a bismuth salt which is combined with a tin derivative reducing agent in an alkaline medium and held together by a binder.

4. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound being a bismuth salt selected from the group consisting of the bismuth salts of inorganic and organic acids and being combined with a reducing agent selected from the group consisting of inorganic and organic tin derivatives.

5. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound being a bismuth salt which is combined with a tin derivative reducing agent in an alkaline medium and held together by a binder selected from the group consisting of cellulose acetate, cellulose acetobutyrate, cellulose nitrate, ethyl cellulose, rubber and chlorinated rubber and ethyl hydroxyethyl cellulose.

6. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, the bismuth compound being a bismuth salt which is combined with a tin derivative reducing agent and a reaction regulator in an alkaline medium and held together by a binder, said reaction regulator being a low melting material selected from the group consisting of benzylthiocyanate, chlorophenol, cinnamyl alcohol, o-cresol, diphenylamine, hexadecanol, hexadecylamine, p-toluidine, triphenyl phosphate, o-vanillin, amino diethanolamine.

7. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound consisting of approximately 2690 parts by weight of bismuth borate, which is combined with the following ingredients in the following approximate parts by weight for applying to said copying sheet: 2500 parts semicarbazide, 2150 parts stannous sulfate anhydrous, 1200 parts diethanolamine, 200 parts cellulose acetate, 300 parts methanol, 1200 parts acetone and 500 parts dichlorethane.

8. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, the bismuth compound consisting of approximately 2610 parts by weight of bismuth oxychloride, which is combined with the following ingredients in the following approximate parts by weight for applying to said copying sheet: 2670 parts tin tartrate, 2000 parts semicarbazide, 2000 parts diphenylamine, 1000 parts di iso propanolamine, 10 parts ethyl cellulose and 2250 parts toluene.

9. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound consisting of approximately 3600 parts by weight of bismuth subsalicylate, which is com-

bined with the following ingredients in the following approximate parts by weight for applying to said copying sheet: 2000 parts tin hydroxide, 1900 parts tri-isopropanolamine, 250 parts polyvinylbutyral, 2500 parts semicarbazide and 2250 parts toluene.

10. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound consisting of approximately 2930 parts by weight of bismuth subnitrate, which is combined with the following ingredients in the following approximate parts by weight for applying to said copying sheet: 2910 parts triethylamine-tin chloride, 2500 parts semicarbazide, 1000 parts ethylparatoluene sulfonate, 200 parts cellulose nitrate and 2300 parts acetone.

11. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound being bismuth lactate, which is combined with the following ingredients in the approximate proportions given for applying to said copying sheet: 36 g. bismuth lactate, 34 g. semicarbazide-tin chloride, 15 g. semicarbazide, 20 g. hydrazine salicylate, 1 g. ethyl hydroxyethyl cellulose, 50 ml. toluene and 400 ml. ligoine.

12. A heat-sensitive copying sheet for producing copies of printed or graphic subject matter by exposure of said sheet, in contact with said subject matter, to radiant energy, said copying sheet having applied thereto the combination of a bismuth compound and a reducing agent capable of reacting with said bismuth compound in the presence of heat to produce metallic bismuth, said bismuth compound being a bismuth salt which is combined with a tin derivative reducing agent in an organic alkaline medium selected from the group consisting of semicarbazide, heterocyclic bases, and the amino- and ethanolamino-derivatives of said heterocyclic bases.

#### References Cited in the file of this patent

#### UNITED STATES PATENTS

|    |           |           |               |
|----|-----------|-----------|---------------|
| 50 | 2,092,566 | Wright    | Sept. 7, 1937 |
|    | 2,663,653 | Zimmerman | Dec. 22, 1953 |
|    | 2,663,656 | Miller    | Dec. 22, 1953 |
|    | 2,740,896 | Miller    | Apr. 3, 1956  |
|    | 2,749,253 | Shoemaker | June 5, 1956  |